# EUROPEAN PATENT APPLICATION

(11) **EP 4 685 249 A1**
(43) Date of publication of application: **28.01.2026**
(21) Application number: 24845419.1
(22) Date of filing: 11.07.2024
(51) Int. Cl.: C21D 6/00, B22D 11/06, B22D 11/16, C22C 38/00, H01F 1/147, H01F 1/153

(54) **IRON-BASED CRYSTAL ALLOY PRODUCTION METHOD**

(30) Priority: 21.07.2023 JP 2023119069
(71) Applicant: Next Core Technologies, Inc., Uji-shi, Kyoto 611-0033 (JP)
(72) Inventor: KANEKIYO, Hirokazu, Kyoto-shi, Kyoto 600-8813 (JP)
(74) Representative: Isarpatent
(86) International application number: PCT/JP2024/025071
(87) International publication number: WO 2025/023038

(57) **Abstract**

A method for producing an iron-based crystal alloy, the method including: a step of preparing an (Fe,Co)-B-based molten alloy 3 having a composition represented by a composition formula (Fe_{1-y}Co_{y})₁₀₀₋ₓ(B_{1-z}C_{z})ₓ and in which x, y, and z satisfy 10.0 ≤ x ≤ 18.0 atom%, 0.05 ≤ y ≤ 0.5, and 0.0 ≤ z ≤ 0.3, respectively; and a quench solidification step of quench-solidifying the molten alloy 3 on a cooling roll 8, wherein the quench solidification step includes a step of injecting the molten alloy 3 onto a surface of the cooling roll 8 from a tapping nozzle 6 while rotating the cooling roll 8 at a roll surface speed of 15 m/sec or more and 40 m/sec or less to fabricate an iron-based crystal alloy 9 in which an abundance ratio of an α-Fe phase is 50 vol% or more and less than 95 vol% and a balance consists of an Fe-B phase. The iron-based crystal alloy is formed in a ribbon shape having a thickness of 50 µm or less, has a saturation magnetic flux density of 1.7 T or more, has an iron loss (W10/1k) of 20 W/kg or less at a magnetic flux of 1.0 T and a frequency of 1 kHz, and has a magnetic permeability of 1500 or more at 1 kHz. An arithmetic average roughness of the surface of the cooling roll 8 is 0.01 µm or more and 0.6 µm or less.

## Description

### Technical Field

The present invention relates to a method for producing an iron-based crystal alloy, and more particularly to a method for producing an iron-based crystal alloy that can be suitably used as a core material applied to a direct current motor.

### Background Art

In recent years, a material having a low iron loss and a high saturation magnetic flux density has been demanded from the market for various passive elements, such as inductors and reactors, and transformers used as electronic components. As such a material, an iron-based amorphous material or an iron-based nanocrystal material containing iron (Fe), silicon (Si), and boron (B) as main raw materials is known, and demand for an Fe-Si-B-based amorphous alloy ribbon having a thickness of about 17 µm to 25 µm fabricated by a molten metal quench solidification method using such a soft magnetic material is increasing mainly for large transformers and inductors as an alternative to a conventional silicon steel sheet.

In addition, since the above Fe-Si-B-based amorphous alloy ribbon has a lower iron loss than that of a silicon steel sheet, it has been studied to improve motor efficiency by applying the Fe-Si-B-based amorphous alloy ribbon to a rotor core and a stator core of a brushless direct current (BLDC) motor by taking advantage of this feature. In particular, when the Fe-Si-B-based amorphous alloy ribbon is used in a high-speed rotation type BLDC motor exceeding 20,000 rpm, since high motor efficiency can be obtained as the operation range of the soft magnetic material becomes a high-frequency band around 2 kHz, it is expected that the Fe-Si-B-based amorphous alloy ribbon is applied to major appliances, such as vacuum cleaners, and electric auxiliary motors that require high-speed rotation of the motor.

On the other hand, a drive motor for EV, which is required to have higher efficiency than that of a motor for major appliances, cannot obtain a required output unless a saturation magnetic flux density (Bs) equivalent to that of a silicon steel sheet can be ensured. Since Bs of the Fe-Si-B-based amorphous alloy is about 1.6 T at the maximum, it is difficult to replace a silicon steel sheet having Bs of 1.7 T or more. For this reason, there has been no example in which an EV drive BLDC motor using the Fe-Si-B-based amorphous alloy has been put on the market.

Regarding an EV drive BLDC motor of several 10 kW or more class, a core material of a silicon steel sheet and an anisotropic rare earth iron-boron-based sintered magnet exhibiting excellent permanent magnet characteristics are combined, and high efficiency by utilizing magnet torque has been conventionally promoted. However, in a silicon steel sheet having a low magnetic permeability, the excellent magnetic characteristics of the anisotropic rare earth iron-boron-based sintered magnet cannot be sufficiently utilized, and thus it is difficult to realize a core material having a low iron loss. For this reason, the market demand for a high-output and high-efficiency BLDC motor capable of contributing to energy saving of automobiles by a synergistic effect of effective use of permanent magnet performance and reduction in iron loss of a core material is extremely high.

Since the Fe-Si-B-based amorphous alloy has a higher magnetic permeability than that of a silicon steel sheet and can reduce the iron loss to about 1/10, an alternative to a silicon steel sheet has been studied as a core material of an EV drive BLDC motor. However, since the saturation magnetic flux density (Bs) is low as described above, the Fe-Si-B-based amorphous alloy is mainly applied to a high-speed rotation type BLDC motor of 15,000 rpm or more in which the influence of iron loss becomes remarkable, and it is difficult to apply the Fe-Si-B-based amorphous alloy to a drive motor for EV having a rotation speed of less than 15,000 rpm. In addition, the Fe-Si-B-based amorphous alloy ribbon has a small thickness of about 25 µm, and it is difficult to perform punching press processing for producing a laminated core or the like for a rotor core and a stator core of a BLDC motor. Therefore, the Fe-Si-B-based amorphous alloy ribbon is mainly limited to use as a wound core, and it is difficult to replace a silicon steel sheet in motor applications.

On the other hand, since an Fe-Si-B-based nanocrystal material is likely to crack or chip, the Fe-Si-B-based nanocrystal material is only used as a wound core or molded after pulverization to be used as a dust core, and it is difficult to use the Fe-Si-B-based nanocrystal material as a laminated core similarly to the Fe-Si-B-based amorphous alloy.

In order to obtain an Fe-Si-B-based amorphous structure or nanocrystal structure, it is necessary to add Si and B, and in order to obtain a nanocrystal structure, an additional element such as Cu or Nb is further required, so that Bs ≥ 1.7 T cannot be obtained due to a decrease in the composition ratio of Fe as a result. For this reason, conventionally, an iron-based alloy that is easy to form a laminated core and can ensure Bs ≥ 1.7 T has not been found.

For example, Non Patent Literature 1 discloses that the quench solidification rate is reduced by adding phosphorus (P), and an iron-based amorphous alloy ribbon having a thickness of 50 µm or more is obtained. However, in the phosphorated alloy, not only the addition of phosphorus causes a decrease in Bs, but also the phosphorus component volatilizes at the time of melting the alloy, so that contamination inside and outside the molten metal quenching apparatus may become significant, and further, the phosphorus component may be likely to burn, and thus there are still few application examples in the industrial field.

Patent Literatures 1 to 3 disclose a method for producing an amorphous alloy ribbon having a plate thickness (e.g., about 50 µm) at which punching processing can be performed by a multi-slit method in which a molten alloy is tapped onto a rotating cooling roll from a plurality of slit nozzles. However, even if such a technique is used, it is difficult to realize Bs ≥ 1.7 T, and it is difficult to apply the material as a soft magnetic material for a laminated core for an EV drive BLDC motor instead of a silicon steel sheet.

Patent Literature 4 discloses a method for producing a metal ribbon in which the thickness of the metal ribbon is suppressed from becoming uneven when a wide quenched ribbon is fabricated using a porous nozzle. The invention of Patent Literature 4 is characterized by the shape of the nozzle opening, but there is a problem that the nozzle processing cost increases due to difficulty in processing, and it is difficult to use the invention at a mass production level.

Patent Literature 5 discloses a method for producing an iron-based silicon boron-based amorphous alloy in which the thickness is increased using a tapping nozzle having a zigzag type multi-orifice, but it is difficult to ensure high Bs and a sufficient thickness as compared with a silicon steel sheet.

Patent Literature 6 discloses an Fe-Si-B-based quench-solidified alloy capable of forming a laminated core characterized by having high Bs of Bs ≥ 1.7 T and a thickness ≥ 40 µm. The invention of Patent Literature 6 is obtained by optimizing the blending ratio of each element in a ternary composition of iron, silicon, and boron, which are essential elements, but since the workability of punching press when a laminated core is produced from an alloy ribbon obtained by this is inferior to that of a silicon steel sheet, there is room for further improvement in fabricating the laminated core at low cost.

### Citation List

### Patent Literature

- Patent Literature 1:: JP H5-329587 A
- Patent Literature 2:: JP H7-113151 A
- Patent Literature 3:: JP H8-124731 A
- Patent Literature 4:: JP S63-220950 A
- Patent Literature 5:: JP 2018-153828 A
- Patent Literature 6:: JP 2021-193199 A

### Non Patent Literature

Non-Patent Literature 1: Creation of a novel bulk metallic glass/amorphous thick plate having a high saturation magnetic flux density (General Research Center for Metallic Glass, TOHOKU University) by Akihiro MAKINO, Ken KUBOTA, and Joshunto

### Summary of Invention

### Technical Problem

An object of the present invention is to provide a method for producing an iron-based crystal alloy capable of easily performing punching processing while ensuring a low iron loss and a high saturation magnetic flux density.

### Solution to Problem

The object of the present invention is achieved by a method for producing an iron-based crystal alloy, the method including: a step of preparing an (Fe,Co)-B-based molten alloy having a composition represented by a composition formula (Fe_{1-y}Co_{y})₁₀₀₋ₓ(B_{1-z}C_{z})ₓ and in which x, y, and z satisfy 10.0 ≤ x ≤ 18.0 atom%, 0.05 ≤ y ≤ 0.5, and 0.0 ≤ z ≤ 0.3, respectively; and a quench solidification step of quench-solidifying the molten alloy on a cooling roll, wherein the quench solidification step includes a step of injecting the molten alloy onto a surface of the cooling roll from a tapping nozzle including a single-slit nozzle while rotating the cooling roll at a roll surface speed of 15 m/sec or more and 40 m/sec or less to fabricate an iron-based crystal alloy in which an abundance ratio of an α-Fe phase is 50 vol% or more and less than 95 vol% and a balance consists of an Fe-B phase, the iron-based crystal alloy is formed in a ribbon shape having a thickness of 50 µm or less, has a saturation magnetic flux density of 1.7 T or more, has an iron loss (W10/1k) of 20 W/kg or less at a magnetic flux of 1.0 T and a frequency of 1 kHz, and has a magnetic permeability of 1500 or more at 1 kHz, and an arithmetic average roughness of the surface of the cooling roll is 0.01 µm or more and 0.6 µm or less.

In the method for producing an iron-based crystal alloy, the tapping nozzle preferably has a slit width of 0.2 mm or more and 0.7 mm or less.

In addition, a distance from the tapping nozzle to the surface of the cooling roll is preferably 0.2 mm or more and 5.0 mm or less.

### Advantageous Effects of Invention

According to the present invention, it is possible to provide a method for producing an iron-based crystal alloy capable of easily performing punching processing while ensuring a low iron loss and a high saturation magnetic flux density.

### Brief Description of Drawings

FIG. 1 is a schematic configuration diagram of an apparatus used in a method for producing an iron-based crystal alloy having a ribbon shape according to an embodiment of the present invention.
FIG. 2 is an enlarged view illustrating a main part of the apparatus illustrated in FIG. 1, in which FIG. 2(a) is a cross-sectional view and FIG. 2(b) is a bottom view.
FIG. 3 is a powder X-ray diffraction profile of an iron-based crystal alloy obtained in one Example of the present invention.
FIG. 4 is a powder X-ray diffraction profile of an iron-based crystal alloy obtained in another Example of the present invention.
FIG. 5 is a powder X-ray diffraction profile of an iron-based crystal alloy obtained in still another Example of the present invention.
FIG. 6 is a powder X-ray diffraction profile of an iron-based crystal alloy obtained in one Comparative Example of the present invention.

### Description of Embodiments

### [Alloy composition]

In order to improve the punching workability of an iron-based alloy, it is necessary to form a crystal structure instead of an amorphous structure, which is hard and likely to crack. The iron-based crystal alloy composition of the present invention is based on a binary alloy composition of Fe-B, in which a part of Fe is substituted with Co, which is a ferromagnetic element like Fe, and the composition formula is represented by (Fe_{1-y}Co_{y})₁₀₀₋ₓ(B_{1-z}C_{z})ₓ.

If the substitution ratio of Co to Fe is too low, it is difficult to realize Bs ≥ 1.7 T, and thus it is necessary to ensure that y in the above composition formula is 0.05 or more. When the value of y increases, Bs of the iron-based crystal alloy monotonically increases up to y = 0.5, but when the value of y exceeds 0.5, Bs does not increase, and only the production cost increases due to use of Co, which is an expensive element. Therefore, 0.05 ≤ y ≤ 0.5 should be satisfied, and 0.1 ≤ y ≤ 0.5 is preferable from the viewpoint of increasing Bs, and 0.15 ≤ y ≤ 0.4 is more preferable in consideration of the production cost.

In the iron-based crystal alloy of the present invention, B is an element essential for obtaining a low iron loss and a high magnetic permeability, and plays a role in forming a structure consisting of an α-Fe phase and an Fe-B phase into a uniform microstructure. A part of B may be substituted with C, and this reduces the melting point of the molten alloy, so that the quench solidification conditions are relaxed, and the iron-based crystal alloy is easily fabricated.

However, if the substitution ratio of C to B is too high, it is difficult to obtain a uniform and fine crystal structure consisting of an α-Fe phase and an Fe-B phase due to generation of an Fe-C compound. Therefore, z in the above composition formula is 0.0 ≤ z ≤ 0.3, and from the viewpoint of maintaining high Bs characteristics, 0.0 ≤ z ≤ 0.2 is preferable, and 0.05 ≤ z ≤ 0.15 is more preferable.

If the ratio of B and C to the overall composition of the iron-based crystal alloy is too low, a coarse α-Fe phase as a starting point of cracking is likely to precipitate during punching press. On the other hand, if the ratio of B and C to the overall composition of the iron-based crystal alloy is too high, an increase in the volume ratio of an Fe-B phase and a decrease in the volume ratio of an α-Fe phase are caused, and it becomes difficult to ensure Bs ≥ 1.7 T. Therefore, x in the above composition formula is 10.0 ≤ x ≤ 18.0 atom%, and 11.0 ≤ x ≤ 17.0 atom% is preferable, and 12.0 ≤ x ≤ 16.0 atom% is more preferable.

### [Metal structure]

The iron-based crystal alloy of the present invention is an (Fe,Co)-B-based iron-based crystal alloy having a composite structure of an α-Fe phase and an Fe-B phase, and has magnetic properties and mechanical properties that greatly contribute to improvement in efficiency of a BLDC motor. If the abundance ratio of the α-Fe phase is too low, it is difficult to ensure Bs ≥ 1.7 T. On the other hand, if the abundance ratio is too high, coarse α-Fe of about 10 µm or more is likely to precipitate, and thus there is a possibility that the coarse α-Fe becomes a starting point of cracking during punching press, and further, an increase in iron loss and a decrease in magnetic permeability are likely to occur. Therefore, the abundance ratio of the α-Fe phase is 50 vol% or more and less than 95 vol%, preferably 60 vol% or more and less than 90 vol%, and more preferably 60 vol% or more and less than 85 vol%. The Fe-B phase is a remaining phase of the α-Fe phase, and is a phase mainly composed of FeB and Fe2B. As described later, the abundance ratio and the crystal grain size of the α-Fe phase can be adjusted to desired values by controlling the quenching rate of the molten alloy. The average crystal grain size of the α-Fe phase is preferably 2 nm to 20 nm. The average crystal grain size of the α-Fe phase can be determined from the half width of an X-ray diffraction peak by powder X-ray diffraction (XRD) described later.

### [Magnetic characteristics]

The saturation magnetic flux density of the iron-based crystal alloy of the present invention is Bs ≥ 1.7 T, but when it is assumed that an EV drive BLDC motor of 30 kW or more is applied, Bs ≥ 1.72 T is preferable, and Bs ≥ 1.75 T is more preferable.

In addition, the iron-based crystal alloy of the present invention has an iron loss (W10/1k) of ≤ 20 W/kg at a magnetic flux of 1.0 T and a frequency of 1 kHz, and has low iron loss performance that is significantly lower than an iron loss (W10/1k) of a silicon steel sheet (JIS standard 35A360) of 96.6 W/kg. When the iron loss (W10/1k) exceeds 20 W/kg, the effect of improving the motor efficiency decreases. In order to further enhance the effect of improving the motor efficiency, an iron loss (W10/1k) of ≤ 15 W/kg is preferable, and an iron loss (W10/1k) of ≤ 10 W/kg is more preferable.

The iron-based crystal alloy of the present invention has a magnetic permeability of 1500 or more at 1 kHz. If the magnetic permeability is lower than 1500 at 1 kHz, the superiority of the magnetic flux amount on the surface of the teeth portion in the stator core over the silicon steel sheet is reduced. In order to further enhance the superiority over the silicon steel sheet, the magnetic permeability is preferably 2000 or more, and more preferably 3000 or more at 1 kHz.

### [Method for producing iron-based crystal alloy]

The iron-based crystal alloy of the present invention is produced by a method for producing an iron-based crystal alloy including a step of preparing an (Fe,Co)-B-based molten alloy having the above composition, and a quench solidification step of quench-solidifying the prepared molten alloy.

FIG. 1 is a schematic configuration diagram of a single-roll molten metal quenching apparatus used in a method for producing an iron-based crystal alloy according to an embodiment of the present invention. The single-roll molten metal quenching apparatus 1 illustrated in FIG. 1 includes a melting furnace 2, a molten metal storage container 5, and a cooling roll 8.

The melting furnace 2 supplies a molten alloy 3 in which a raw material is melted by high-frequency induction heating to the molten metal storage container 5 by rotation of a tilting shaft 4. The molten metal storage container 5 includes a tapping nozzle 6 at the bottom, further heats the molten alloy 3 by a heating coil (not illustrated), and jets the molten alloy 3 from a slit 7 formed at the lower end of the tapping nozzle 6 to the surface (outer peripheral surface) of the cooling roll 8. When cooling water is supplied to the inside of the cooling roll 8, the molten alloy in contact with the surface is quenched to form an (Fe,Co)-B-based quench-solidified alloy 9 having a ribbon shape. The material of the tapping nozzle 6 can be appropriately selected from, for example, quartz (SiO₂), boron nitride (BN), silicon carbide (SiC), and alumina (Al₂O₃).

FIG. 2 is an enlarged view illustrating the tapping nozzle 6 of the apparatus illustrated in FIG. 1, in which FIG. 2(a) is a cross-sectional view and FIG. 2(b) is a bottom view. The tapping nozzle 6 illustrated in FIG. 2(a) is a single-slit nozzle in which a single slit 7 is formed. The width W1 of the slit 7 serves to adjust the tapping rate of the molten alloy 3 supplied to the cooling roll 8. If the slit width W1 is too small, slit processing is likely to be difficult, and further, the slit 7 is likely to be blocked by the molten metal. On the other hand, if the slit width W1 is too large, the tapping rate becomes too high, heat extraction in the cooling roll 8 cannot be performed in time, and the quench-solidified alloy sticks to the cooling roll 8, so that it is difficult to continue stable molten metal quench solidification. Therefore, the slit width W1 is 0.2 mm or more and 0.7 mm or less. The slit width W1 is preferably 0.3 mm or more and 0.6 mm or less, and more preferably 0.3 mm or more and 0.5 mm or less.

The molten metal supplied to the surface of the cooling roll 8 becomes the quench-solidified alloy 9 having a ribbon shape by rotation of the cooling roll 8, and is peeled off from the cooling roll 8. If the surface speed of the cooling roll 8 is too low, an (Fe,Co)-B-based quench-solidified alloy having an excessive thickness exceeding 50 µm is formed, so that a coarse α-Fe phase precipitates, and cracking is likely to occur during punching press. On the other hand, if the surface speed of the cooling roll 8 is too high, miniaturization of the (Fe,Co)-B-based crystal alloy proceeds too much, and the abundance ratio of an α-Fe phase decreases, so that it tends to be difficult to ensure Bs ≥ 1.7 T. Therefore, the surface speed of the cooling roll 8 is 15 m/sec or more and 40 m/sec or less, preferably 15 m/sec or more and 35 m/sec or less, and more preferably 17 m/sec or more and 32 m/sec or less. The diameter of the cooling roll 8 is, for example, 200 to 20000 mm. Water cooling is not necessarily required for the cooling roll 8 as long as the quench solidification time is a short time of 10 sec or less. However, when the quench solidification time is 10 sec or more, it is preferable to suppress the temperature rise of the surface of the cooling roll 8 by allowing cooling water to flow inside the cooling roll 8. The water cooling capacity of the cooling roll 8 is preferably appropriately adjusted according to the latent heat of solidification per unit time and the tapping rate.

In the fabrication of the quench-solidified alloy 9 having a ribbon shape, the adhesion of the molten alloy 3 to the outer surface of the cooling roll 8 is important, and the molten metal adhesion largely depends on the surface roughness of the cooling roll 8. If the surface roughness of the cooling roll 8 is too small, the molten alloy 3 slides on the surface of the cooling roll 8, so that sufficient cooling becomes difficult. On the other hand, if the surface roughness of the cooling roll 8 is too large, there is a possibility that the quenched alloy sticks to the cooling roll 8. Therefore, the arithmetic average roughness (Ra) of the surface of the cooling roll 8 is 0.01 µm or more and 0.6 µm or less, preferably 0.05 µm or more and 0.55 µm or less, and more preferably 0.1 µm or more and 0.5 µm or less.

In FIG. 1, if the distance d from the tip of the tapping nozzle 6 to the surface of the cooling roll 8 is too small, the quenched alloy sticks to the cooling roll 8, and there is a possibility that stable quench solidification of the molten alloy 3 cannot be continued. On the other hand, if the distance d is too large, a lump of molten metal (puddle) is not formed on the surface of the cooling roll 8, and there is a possibility that quench solidification of the molten alloy 3 cannot be performed. Therefore, the above distance d is 0.2 mm or more and 5.0 mm or less, preferably 0.3 mm or more and 3.0 mm or less, and more preferably 0.3 mm or more and 2.0 mm or less.

The cooling roll 8 is preferably excellent in thermal conductivity and durability by being formed of a material containing any one of pure copper, a copper alloy, molybdenum (Mo), and tungsten (W) as a main raw material. The main raw material means that the material accounts for 50% or more by weight. The surface of the cooling roll 8 may be plated with chromium, nickel, or an alloy thereof, thereby being able to increase the heat resistance and hardness of the surface of the cooling roll 8 and to suppress melting and deterioration of the surface of the roll during quench solidification.

### [Heat treatment]

In a preferred embodiment, an (Fe,Co)-B-based quench-solidified alloy is heat-treated at a constant temperature of 200°C or more and 700°C or less, so that strain in the quench-solidified alloy can be removed, and further reduction in iron loss can be realized. If the heat treatment temperature is lower than 200°C, the effect of strain removal is small. If the heat treatment temperature exceeds 700°C, coarsening of an α-Fe phase proceeds, so that brittleness of the quench-solidified alloy increases, and the quench-solidified alloy is likely to crack during punching processing. The above heat treatment temperature is preferably 300°C or more and 700°C or less, and more preferably 400°C or more and 680°C or less. The heat treatment time of the above heat treatment depends on the shape of the soaking zone of the heat treatment apparatus, and an optimum heat treatment time is appropriately selected within a time range of 3 minutes or more and less than 2 hours. The above heat treatment is preferably performed in a vacuum or inert gas atmosphere, but heat treatment in the atmosphere is also allowed.

### Examples

Hereinafter, the present invention will be described more specifically with reference to Examples. However, the present invention is not limited to the following Examples.

In an alumina crucible (melting furnace), 100 kg of a raw material in which respective elements of B, C, Co, and Fe having a purity of 99.5% or more were blended so as to have an alloy composition shown in Examples 1 to 11 and Comparative Examples 12 to 17 in the following Table 1 was housed, and was melted by high-frequency induction heating to form a molten alloy. Fifty kilograms (50 kg) of the molten alloy was poured into a molten metal storage container made of alumina having an inner diameter of 200 mm × a height of 400 mm and including a BN tapping nozzle having a slit shown in Table 1 at the bottom. The slit width and the slit length of the tapping nozzle are as shown in Table 1.

Thereafter, 50 kg of the molten alloy was further heated by energizing a high-frequency heating coil installed around the molten metal storage container, and after the temperature of the molten alloy reached a temperature higher than the melting point of the blended composition alloy by 100°C or more, an alumina molten metal stopper disposed above the tapping nozzle was pulled out. As a result, the molten alloy was jetted from the tapping nozzle to the surface of the cooling roll immediately below. The cooling roll is made of chromium zircon copper, and has an outer diameter of 600 mm and a width of 200 mm. In addition, the gap between the tapping nozzle and the surface of the cooling roll is as shown in Table 1. In addition, the injection pressure of the molten alloy from the tapping nozzle, the roll surface speed of the cooling roll, and the arithmetic average roughness (Ra) of the roll surface of the cooling roll are as shown in Table 2.

The molten alloy jetted onto the surface of the cooling roll formed a lump of molten metal (puddle) on the surface of the cooling roll, and was quench-solidified at the interface between the puddle and the cooling roll to obtain a quench-solidified alloy having a ribbon shape and an average thickness and an average width shown in Table 3. In Example 3, the quench-solidified alloy was subjected to heat treatment at 650°C for 10 minutes in an Ar flow gas. When the quench-solidified alloy thus obtained was subjected to a punching test, the results shown in Table 3 were obtained.

The quench-solidified alloy thus obtained was subjected to structure evaluation by powder X-ray diffraction (XRD), and as a result, the quench-solidified alloys of Examples 1 to 11 were all crystal alloys consisting of α-Fe type and Fe-B type compounds. The vol% of α-Fe precipitated in the quench-solidified alloy (the abundance ratio of α-Fe was determined by X-ray diffraction) is shown in Table 3. Quantitative analysis of constituent phases by powder X-ray diffraction is a general evaluation method, and is incorporated into analysis software of an X-ray diffractometer, and it is possible to grasp the composition ratio of each phase. As representative examples of the powder X-ray diffraction profiles of the quench-solidified alloys of Examples, Examples 4 and 9 are shown in FIGS. 3 and 4, respectively. As shown in FIGS. 3 and 4, the structures of the quench-solidified alloys of Examples 4 and 9 were composite structures consisting of an α-Fe phase and an Fe-B phase.

Bs, iron loss, and magnetic permeability of the as-spun (immediately after quench solidification) quench-solidified alloys or the quench-solidified alloys after heat treatment of Examples 1 to 11 and Comparative Examples 12 to 17 are shown in Table 4. Bs was measured using a vibrating sample magnetometer manufactured by Toei Industry Co., Ltd., and iron loss and magnetic permeability were measured using a B-H analyzer manufactured by Iwatsu Electric Co., Ltd. As described above, only the quench-solidified alloy of Example 3 was subjected to heat treatment, and as shown in FIG. 5, the powder X-ray diffraction profile of the quench-solidified alloy of Example 3 was also a composite structure consisting of an α-Fe phase and an Fe-B phase.

The quench-solidified alloys of Comparative Examples 12 to 17 had a metal structure of an amorphous single phase as evaluated by powder X-ray diffraction (XRD). Table 3 shows the vol% of α-Fe (the abundance ratio of α-Fe was determined by X-ray diffraction). As a representative example of the powder X-ray diffraction profiles of the quench-solidified alloys of Comparative Examples, Comparative Example 12 is shown in FIG. 6. As shown in FIG. 6, the structure of the quench-solidified alloy of Comparative Example 12 was an amorphous single phase structure.

### Reference Signs List

- 1: single-roll molten metal quenching apparatus
- 2: melting furnace
- 3: molten alloy
- 4: tilting shaft
- 5: molten metal storage container
- 6: tapping nozzle
- 7: slit
- 8: cooling roll
- 9: quench-solidified alloy

## Claims

1. method for producing an iron-based crystal alloy, the method comprising:
a step of preparing an (Fe,Co)-B-based molten alloy having a composition represented by a composition formula (Fe_{1-y}Co_{y})₁₀₀₋ₓ(B_{1-z}C_{z})ₓ and in which x, y, and z satisfy 10.0 ≤ x ≤ 18.0 atom%, 0.05 ≤ y ≤ 0.5, and 0.0 ≤ z ≤ 0.3, respectively; and
a quench solidification step of quench-solidifying the molten alloy on a cooling roll,
wherein the quench solidification step includes a step of injecting the molten alloy onto a surface of the cooling roll from a tapping nozzle including a single-slit nozzle while rotating the cooling roll at a roll surface speed of 15 m/sec or more and 40 m/sec or less to fabricate an iron-based crystal alloy in which an abundance ratio of an α-Fe phase is 50 vol% or more and less than 95 vol% and a balance consists of an Fe-B phase,
the iron-based crystal alloy is formed in a ribbon shape having a thickness of 50 µm or less, has a saturation magnetic flux density of 1.7 T or more, has an iron loss (W10/1k) of 20 W/kg or less at a magnetic flux of 1.0 T and a frequency of 1 kHz, and has a magnetic permeability of 1500 or more at 1 kHz, and
an arithmetic average roughness of the surface of the cooling roll is 0.01 µm or more and 0.6 µm or less.

2. The method for producing an iron-based crystal alloy according to claim 1, wherein the tapping nozzle has a slit width of 0.2 mm or more and 0.7 mm or less.

3. The method for producing an iron-based crystal alloy according to claim 1 or 2, wherein a distance from the tapping nozzle to the surface of the cooling roll is 0.2 mm or more and 5.0 mm or less.
